



US005372610A

**United States Patent** [19]**Kahle et al.****Patent Number:** 5,372,610**Date of Patent:** Dec. 13, 1994

[54] **PROCESS FOR THE AFTER-BLEACHING OF DYED RAW CELLULOSE USING CATIONIC COMPOUNDS**

[75] Inventors: **Volker Kahle**, Bergisch Gladbach; **Klaus Kackstädter**; **Karl-Heinz Passon**, both of Leverkusen; **Martin Riegels**, Hilden; **Klaus Walz**, Leverkusen, all of Germany

[73] Assignee: **Bayer Aktiengesellschaft**, Leverkusen, Germany

[21] Appl. No.: 940,117

[22] Filed: Sep. 3, 1992

[30] **Foreign Application Priority Data**

Sep. 13, 1991 [DE] Germany ..... 4130484

[51] Int. Cl.<sup>5</sup> ..... D06L 3/02

[52] U.S. Cl. ..... 8/111; 8/102

[58] Field of Search ..... 252/182.3, 186.29; 8/111, 102

[56] **References Cited**

**U.S. PATENT DOCUMENTS**

3,996,151 12/1976 Kirner .

4,510,068 4/1985 Rohlf et al. ..... 252/186.29

4,515,596 5/1985 Berendt et al. ..... 8/107  
4,880,566 11/1989 Baehr et al. .  
4,959,075 9/1990 Baehr et al. .  
5,180,514 1/1993 Farr et al. ..... 8/111 X

**FOREIGN PATENT DOCUMENTS**

0100300 7/1983 European Pat. Off. .  
2301627 9/1976 France .  
3545909 6/1987 Germany .  
0472179 4/1972 U.S.S.R. .

*Primary Examiner*—Johann Richter

*Assistant Examiner*—Michael B. Hydorn

*Attorney, Agent, or Firm*—Sprung Horn Kramer & Woods

[57]

**ABSTRACT**

Dyed raw cellulose can be bleached in a bleaching and after-treatment bath containing, in addition to usual stabilizers, cationic-monomeric and/or polymeric compounds and, if desired, nonionic surfactants. Bleaching is carried out with the aid of aqueous-hydrogen peroxide. The stabilizers that can be used and the cationic compounds are defined in the specification. Nonionic tensides, if their co-use is desired, are those of the class polyglycolethers.

**4 Claims, No Drawings**

**PROCESS FOR THE AFTER-BLEACHING OF  
DYED RAW CELLULOSE USING CATIONIC  
COMPOUNDS**

**BACKGROUND OF THE INVENTION**

**1. FIELD OF THE INVENTION**

The invention relates to a process for the bleaching of raw cellulose, preferably raw cotton, materials dyed with direct or reactive dyestuffs in a bleaching and after-treatment bath, characterised in that this bath contains

- a) stabilisers,
- b) cationic monomeric and/or polymeric compounds and, if desired,
- c) a non-ionic surfactant,
- and the bleaching auxiliaries comprising components a), b) and c).

Textile materials made of cellulose fibres are subjected, according to the prior technique, during pretreatment for dyeing, to a bleaching process, for example using hydrogen peroxide, in alkaline medium. This is followed by drying, dyeing and washing the bleached material.

The large number of steps in the pretreatment, such as, for example, boiling, washing, bleaching and drying, are time-consuming and cost-intensive steps in the textile industry. There have already been many attempts to carry out the processes described above in a simpler and less costly manner.

**2. DESCRIPTION OF THE RELATED ART**

EP 0,100,300 describes a process for the after-treatment of dyed, non-pre-bleached cellulose-containing fibre materials in a combined washing and bleaching bath. The treatment bath contains the following components:

- a) derivatives of phosphonic or phosphorous acid as stabilisers and, if desired,
- b) polyhydroxy compounds.

It is already known (cf. SU 472,179) to dye and bleach cellulose textiles at the same time. The treatment liquor contains Cubosol dyestuffs, sodium nitrite, wetting agents and hydrogen peroxide stabilised with sodium metasilicate. Fixation of the dyestuff and bleaching take place simultaneously in a saturated steam atmosphere at 100° to 101° C. over a period of 3 to 10 minutes.

However, even these processes were not able to fully meet the demands in practice.

**SUMMARY OF THE INVENTION**

It has now been found that bleaching of cellulose materials dyed with direct or reactive dyestuffs can be carried out while achieving optimum properties in practical application by carrying out the treatment of such materials in a bleaching and after-treatment bath containing the following components:

- a) stabilisers for the aqueous hydrogen peroxide bleaching liquors
- b) cationic monomeric compounds and/or cationic polymers or polycondensation products and, if desired,
- c) non-ionic surfactants.

The invention furthermore relates to the bleaching auxiliaries mentioned comprising components a), b) and, if desired, c).

**DETAILED DESCRIPTION OF THE  
INVENTION**

The bleaching auxiliaries can contain

- a) 10-60% by weight of one or more stabilisers,
  - b) 10-60% by weight of one or more cationic agents and
  - c) 0 to 30% by weight of one or more non-ionic surfactants, preferably
- a) in an amount of 30-45% by weight,
  - b) in an amount of 30-45% by weight and
  - c) in an amount of 10-25% by weight.

The bleaching liquor stabilisers as such are known as prior art to one skilled in the art and described, for example, in Chwala/Anger "Handbuch der Textilhilfsmittel" (Handbook of Textile Auxiliaries), edition 1977, from page 340 onwards. Suitable bleaching liquor stabilisers are the following classes of compounds:

- a1) phosphorus compounds, such as tripolyphosphates, orthophosphates, phosphonic acids, such as hydroxyethane-1,1-diphosphonic acid and phosphonoalkane-polycarboxylic acids, and 2-phosphonobutane-1,2,4-tricarboxylic acid (cf. DE 2,061,838, EP 0,100,300)
- a2) magnesium salts of aminopolycarboxylic acids (German Auslegeschrift 1,113,931)
- a3) ethylenediaminetetraacetic acid and salts thereof
- a4) polyacrylic acids and derivatives
- a5) gluconic acid
- a6) polyaminopolycarboxylic acid
- a7) polycarboxylic acid
- a8) (poly)aminomethylenephosphonic acids
- a9) sodium sulphamate (DE 3,342,175)
- a10) aspartic acid
- a11) sulphosalicylic acid
- a12) polyhydroxamic acids
- a13) sodium silicate and magnesium silicate
- a14) phosphonic ester oligomers (EP 82,823).

In most cases, the stabilisers contain mixtures of the active compounds listed above, such as, for example: gluconic acid and sodium pyrophosphate

polyacrylamide, hexametaphosphate and orthophosphate

sodium gluconate and sodium ethylenediaminetetraacetate

ethylenediaminetetraacetic acid and hydroxyethane-1,1-diphosphonic acid

gluconic acid, 2-phosphonobutane-1,2,4-tricarboxylic acid and ethylenediaminetetraacetic acid.

Suitable cationic agents are monomeric and polymeric compounds containing at least 1 cationic nitrogen; in particular quaternary compounds.

The group of cationic compounds includes, for example:

- b1) alkylamine salts
- b2) quaternary ammonium salts
- b3) alkylpyridinium salts
- b4) protonated imidazole compounds or quaternary imidazolinium salts thereof
- b5) alkyldiamines and alkylpolyamines and quaternisation products thereof
- b6) acyldiamines and acylpolyamines and quaternisation products thereof
- b7) methyleneoxyalkylpyridinium salts and
- b8) alkylethyleneureas.

Compounds of this type are sufficiently well-known in the art. Some of them are used as levelling agents for

the dyeing of anionic polyacrylonitrile fibres (cf. R. Rohkohl, Tenside 2 (1965) 76).

Further suitable compounds of group b) are

b9) cationic polymers and polycondensation products, such as often used in the paper and textile industry, for example described in:

Aftertreatments for improving the fastness of dyes on textile fibers, C. C. Cook, Rev. Prog. Coloration 12 (1982) 73 and

H. Fischer: Textilveredlung 25 (1990), pages 54 to 61.

Some examples of the cationic monomeric and polymeric compounds according to the invention are described below:

cationic monomeric compounds of the following formula



where

R and R<sup>1</sup> are C<sub>1</sub>-C<sub>20</sub>-alkyl, C<sub>3</sub>-C<sub>20</sub>-alkenyl, cycloalkyl, aralkyl,

R<sup>2</sup> and R<sup>3</sup> are C<sub>1</sub>-C<sub>4</sub>-alkyl, C<sub>1</sub>-C<sub>4</sub>-hydroxyalkyl or both radicals, together with N, form a heterocyclic ring,

R<sup>4</sup> is —CO—NH—alkylene (C<sub>2</sub>-C<sub>3</sub>) —COO—alkylene (C<sub>2</sub>-C<sub>3</sub>) —CH(OH)—CH<sub>2</sub>—O—alkylene (C<sub>2</sub>-C<sub>3</sub>) —O—CH<sub>2</sub>—CH(OH)—CH<sub>2</sub>—

where

m+n is 0 or 1

X<sup>⊖</sup> is an anion,

the cationic polymers are described by the following formulae:

structural units



where

R<sup>5</sup> is H, C<sub>1</sub>-C<sub>4</sub>-alkyl, C<sub>1</sub>-C<sub>4</sub>-hydroxyalkyl

R<sup>6</sup> is R<sup>5</sup> cyclohexyl, benzyl

R<sup>7</sup> is C<sub>2</sub>-C<sub>12</sub>-alkylene, which may be interrupted by one or more



or structural units



where

R<sup>8</sup> is



or polydiallyldimethylammonium chloride dicyandiamide/formaldehyde/ammoniumchloride condensation products.

The non-ionic surfactants used are polyglycol ethers, for example EO/PO copolymers, sugar polyethers and alkoxylation products, in particular ethoxylation products of fatty alcohols, fatty amines, phenol-styrene adducts, alkylphenols, fatty acids and fatty amides. The surfactants contain 4 to 100 alkenoxy groups, in particular 12 to 60 ethyleneoxy groups.

The ratio of components a):b):c) is 1:0.5-3.0:0.00-1.0, in particular 1:0.7-2.5:0.1-0.8.

Cellulose-containing fibre materials can be dyed by the process according to the invention without pretreatment and then bleached in alkaline medium.

The process according to the invention prevents bleeding of the dyestuff into the bleaching bath to the greatest possible extent and thus makes it possible to use the liquor repeatedly for differently dyed fibre materials.

If dyed raw cotton is subjected to a standard bleaching process, bleeding of dyestuffs into the bleaching liquor necessarily leads to a loss in colour depth. The new process makes it possible to use smaller amounts of dyestuff, since the components according to the invention virtually prevent bleeding of the dyestuffs during the after-bleaching process. The cellulose-containing fibre materials used are dyed in the customary liquors using direct or reactive dyestuffs, such as known in practice.

Preferably, this process can be carried out, for economic reasons, as a wet-on-wet process.

The advantages of this process compared with conventional ones are as follows:

Depending on the reactive dyestuffs and processes used, a yield which is higher by up to 80% and higher brilliance of the dyeings are obtained. Staining of the bleaching liquors is also substantially reduced. This enables, for example, different shades to be after-bleached in the same bleaching liquor. In this way, the economy of the underliquor bleach systems is substantially increased.

The after-bleaching process of raw cotton dyed with reactive or direct dyestuffs is carried out in the usual manner.

The amounts used of the mixtures mentioned vary within wide limits and depend, inter alia, on the process, the bleaching level to be achieved, etc.

A rough classification can be made as follows:



0.50% of C. I. Reactive Blue 116.

It is then subjected to hot rinsing at 60° C. for 10 minutes. Bleaching is started at 60° C. by adding

0.5 ml/l of the reaction product of decyl alcohol with 5 ethylene oxide and 4 propylene oxide

5

2.0 ml/l of mixture B

1.2 g/l of 100% NaOH

3.0 ml/l of 50% strength H<sub>2</sub>O<sub>2</sub>.

The liquor is heated to 90° C. at a gradient of 2° C./min. At this temperature, the piece is treated for 30 minutes. The liquor is dropped and the piece is soaped at the boil for 10 minutes with addition of 0.5 ml/l of a 50% strength solution of 2-phosphonobutane-1,2,4-tricarboxylic acid and 0.5 ml/l of an anionic detergent. Finally, it is rinsed hot and cold.

Bleaching carried out by this process is distinguished by a colour depth which is 30% higher than in bleaching without the auxiliaries according to the invention.

Instead of the polycondensation product used in mixture B, products having recurring units of the following 20 formulae



15



25



30

or a product prepared by polycondensation of dicyandiamide, formaldehyde and ammonium chloride can also be used equally successfully.

What is claimed is:

1. In a process for the bleaching of cellulose materials dyed with direct or reactive dyestuffs, whereby bleaching is carried out with aqueous hydrogen peroxide bleaching liquors comprising the steps of (i) dyeing the raw cellulose, (ii) treating the dyed-raw cellulose in a combined washing and bleaching bath, and (iii) drying, 45

35

b1) alkylamine salts; b2) quaternary ammonium salts; b3) alkylpyridinium salts; b4) protonated imidazole compounds or quaternised imidazolium salts thereof; b5) alkyldiamines and alkylpolyamines and quaternisation products thereof; b6) acyldiamines and acylpolyamines and quaternisation products thereof; b7) methyleneoxyalkylpyridinium salts; b8) alkylethyleneureas; and b9) cationic polymers and polycondensation products.

4. The process of claim 1, wherein the ratio of a):b):c) is a weight ratio of 1:0.7-2.5:0.1-0.8.

\* \* \* \* \*

the improvement which comprises carrying out said treating and bleaching steps in a bleaching and after-treatment bath containing the following components:

a) stabilisers for the aqueous hydrogen peroxide bleaching liquors,

b) one or more members selected from the group consisting of cationic monomeric compounds, cationic polymers and polycondensation products, and, if desired,

c) polyglycolether surfactants.

2. The process of claim 1, wherein said stabilizers comprise one or more compound(s) from the following classes of compounds:

a1) tripolyphosphates, orthophosphates, phosphonic acids, phosphonoalkane-polycarboxylic acids;

a2) magnesium salts of aminopolycarboxylic acids;

a3) ethylenediaminetetraacetic acid and salts thereof;

a4) polyacrylic acids and derivatives;

a5) gluconic acid;

a6) polyaminopolycarboxylic acid;

a7) polycarboxylic acid;

a8) (poly)aminomethylenephosphonic acids;

a9) sodium sulphamate;

a10) aspartic acid;

a11) sulphosalicylic acid;

a12) polyhydroxamic acids;

a13) sodium silicate and magnesium silicate; and

a14) phosphonic ester oligomers.

3. The process of claim 1, wherein said one or more members selected from the group consisting of cationic monomer compounds, cationic polymers, and polycondensation compounds are one or more compound(s) from the following classes of compounds:

b1) alkylamine salts;

b2) quaternary ammonium salts;

b3) alkylpyridinium salts;

b4) protonated imidazole compounds or quaternised imidazolium salts thereof;

b5) alkyldiamines and alkylpolyamines and quaternisation products thereof;

b6) acyldiamines and acylpolyamines and quaternisation products thereof;

b7) methyleneoxyalkylpyridinium salts;

b8) alkylethyleneureas; and

b9) cationic polymers and polycondensation products.

55